

## UNITED STATES PATENT OFFICE

2,272,556

## COLORING PHOTOGRAPHIC IMAGES

Alan M. Gundelfinger, Los Angeles, Calif., assignor to Cinecolor, Incorporated, Los Angeles, Calif., a corporation of California

No Drawing. Application December 20, 1938.  
Serial No. 246,810

3 Claims. (Cl. 95—88)

My invention relates generally to color photography, and has particular reference to the production of metallic-toned images that are both fine-grained and well-defined in appearance. In many instances and particularly where sound track images are to be colored, it is quite essential that the images be as sharply defined as possible, but it has been found that the conditions which make for good definition produce an image which is distinctly grainy in appearance.

In motion picture work, where the images are to be greatly magnified by projection on a screen, graininess is very undesirable since it materially detracts from the pleasing appearance of the picture. Furthermore, excessive graininess in sound track images reduces the quality of their sound reproduction.

This problem of graininess versus definition is always present when it is desired to tone the sound track images and one or more component picture images simultaneously with the same solution. For example, for many reasons it is often desirable to use an iron tone to color both the blue component images in a picture and their accompanying sound track in one step, and I have found that when the toning solution is adjusted to give slightly diffused pictures which have but little apparent grain, the definition of the sound track images is not sufficiently good to secure faithful reproduction of the sound recorded on the film. Conversely, when the iron toning solution is adjusted to give excellent definition and consequently good sound reproduction, the images will exhibit such apparent graininess as to be unsatisfactory.

It is, therefore, the major object of my invention to overcome these obstacles, and to provide a process of toning photographic images whereby the images are diffusely colored throughout their image area, and are thus satisfactory for picture projection, which said images also have unusually good definition, and are therefore capable of giving optimum sound reproduction quality.

One suitable method for accomplishing the object of this invention is disclosed and claimed in the joint application of Lyne S. Trimble and myself, Serial No. 246,848, and it is the purpose of this invention to provide an additional method of producing a colored photographic image which is satisfactory, both as to diffusion and definition.

In general, I accomplish my object by first treating the silver image with a toning solution which has been adjusted to give a diffused image, that is to say, the tone is of such character that a certain amount of bleeding or diffusion of the

color throughout the gelatin in the immediate vicinity of the salt grains forming the image will be had. This bleeding or diffusion of the color within the image area colors the gelatin between the salt grains and causes the image to present a more or less uniform colored appearance. However, in using such a tone, the color also bleeds outwardly from the image, and thus creates a halo or fringe of diffused color entirely surrounding the image proper.

In the specification and claims, the term "image" will be used to denote the original image area defined by free silver in the first instance and metallic salt grains subsequently, and the term "fringe" will be used to denote the diffused outline surrounding the image proper, it being understood that the term "diffused image" wherever used herein means an image formed of colored grains, whose color has bled into the surrounding emulsion between and among the grains to give a more or less uniformly colored image without apparent graininess.

In the preferred form of my invention, a photographic silver image is first produced by exposure and development of a light sensitive silver salt in conventional manner, and is then toned with a suitable metallic tone, for example an iron toning solution, such as the following:

|    |                           |       |    |
|----|---------------------------|-------|----|
| 30 | Ferric ammonium oxalate   | grams | 6  |
|    | Potassium ferricyanide    | do    | 6  |
|    | Ammonium chloride         | do    | 10 |
|    | Hydrochloric acid (conc.) | cc    | 5  |
|    | Water to make             | liter | 1  |

35 This treatment converts the silver image to a Prussian Blue image which is generally considered to be ferric ferrocyanide and/or a double salt of ferric ferrocyanide and an alkali metal ferrocyanide, and in either case the image contains a silver salt when first formed. In solutions, such as the one above containing a halide, the silver salt in the resulting Prussian Blue image will be a silver halide, but if a toning solution is used which does not contain a halide, the silver is in the form of silver ferrocyanide.

As previously mentioned, it is possible to control the amount of diffusion and thereby the amount of fringing in the toned image by controlling the amount of available iron in the toning solution, and I have found that the degree of diffusion varies directly as the ratio of ferricyanide ion concentration to ferric ion concentration in the toning solution. The exact proportions of the various constituents of the toning solution and the precise ratio between ferricyanide and

ferric ion concentrations may be varied between comparatively wide limits, depending upon the type of emulsion used, the density of the images, the type of image desired, and the other steps of the general color process. It is to be borne in mind, however, that the toning solution must be adjusted so as to give images which are sufficiently diffused to be satisfactory for picture projection which means, of course, that a definite fringe will be produced.

After the image has been toned, the film is preferably washed and is then treated with a solution capable of eliminating the fringe, this treatment being continued until the fringe is substantially eliminated, care being taken, however, to stop the treatment before the color or the structure of the image is materially modified. By this elimination of the fringe, good definition is restored to the image without apparent graininess. In the process of said previously-mentioned copending application, best results are obtained by holding the pH of the second treating solution, therein named, generally between about 6.5 and 7.5, and if the pH in that process is raised much above 8, considerable difficulty is experienced in controlling the reactions and successfully accomplishing the purposes of the process.

I have now discovered that the fringe can be removed by treating the film with a solution having a relatively high pH value and that the treatment can be controlled within reasonable limits if the reactions mentioned in my said copending application are either absent or kept down to a minimum. In other words, if the Prussian Blue image is treated with a strongly alkaline solution with a pH above 8, and preferably in the vicinity of 9 or 10, direct conversion of substantially all of the Prussian Blue in the fringe and some of the Prussian Blue in the image proper to ferric hydroxide is accomplished.

The rate of this reaction depends upon the pH of the solution used, or to put it conversely, the pH value chosen depends upon the time allowed for film treatment. The permissible upper limit of the pH depends principally upon the characteristics of the film, since as is well-known, the ordinary photographic emulsion cannot stand treatment with a solution which is too alkaline. The lower limit of the pH must of course be above 7.0 and from a practical standpoint must be above 8.0, since below that point, the treating time is much too long. As mentioned, I prefer a pH between 9 and 10, since with the usual emulsion and blue tone this solution will substantially eliminate the fringe in approximately 3 minutes without materially affecting the image.

Various substances may be employed to furnish the OH ions for the conversion; for example, strongly alkaline salts such as sodium or potassium carbonate, tri-sodium phosphate, or the like, or the usual hydroxide of sodium, potassium, ammonia, etc.

After the conversion to ferric hydroxide has been sufficiently effected as above described, the hydroxide is removed by acid treatment, which may take the form of a separate step, or may be combined with the washing step by acidifying the wash water, or in some cases if the subsequent solutions used in the color process are acid, the

fringe may be left in the hydroxide form until the film is immersed in the subsequent treating solution and will be then removed by the acid therein.

5 The ferric ferrocyanide which diffuses out from the agglomerated grains of the image is in a colloidal or highly dispersed state, and is therefore more readily attacked by the OH ions than are the grains themselves. Hence, the amount of 10 ferric ferrocyanide in the fringe is much less than in the image proper, and the preponderance of OH ions in the gelatin of the fringe is so great that they are but little depleted by reaction with the ferric ferrocyanide which means that the 15 reaction goes substantially to completion. However, in the image proper, due to the greater concentration of the ferric ferrocyanide therein, it greatly preponderates over the OH ions entering that part of the gelatin, and hence the OH ions 20 entering the main body of the image are rapidly depleted before a noticeable amount of the ferric ferrocyanide has been converted. Consequently, if the treatment is stopped when the color has disappeared from the fringe, there still will be no appreciable modification of the color or structure 25 of the image proper, although the overall density will be a trifle lighter.

As previously mentioned, it is highly desirable that no reducing agent be employed in the second treating solution, since the reactions described in said copending application proceed simultaneously with the conversion of the Prussian Blue to ferric hydroxide and the reactions become uncontrollable, there being danger of seriously modifying or impairing the color of the image proper.

I claim as my invention:

1. The method of coloring a metallic photographic image which includes: treating said image with an iron toning solution comprising a soluble ferricyanide and a soluble ferric salt to produce a diffused Prussian Blue image having a fringe; and then treating said image with a solution having a pH above 8.0 until said fringe is substantially eliminated but the color of said image is not materially modified.

2. The method of coloring a metallic photographic image which includes: treating said image with an iron toning solution comprising a soluble ferricyanide and a soluble ferric salt to produce a diffused Prussian Blue image having a fringe; and then treating said image with a solution whose pH is maintained between approximately 8.0 and 10.5 until said fringe is substantially eliminated but the color of said image is not materially modified.

3. The method of coloring a metallic photographic image which includes: treating said image with an iron toning solution comprising a soluble ferricyanide and a soluble ferric salt to produce a diffused Prussian Blue image having a fringe; and then treating said image with a solution which is sufficiently alkaline to convert ferric ferrocyanide to ferric hydroxide but which will not reduce the ferric ions in Prussian Blue to ferrous ions, until said fringe is substantially eliminated but the color of said image is not materially modified.

ALAN M. GUNDELFINGER.